

## UNITED STATES PATENT OFFICE

LEO H. BAKELAND, OF YONKERS, NEW YORK, ASSIGNOR TO BAKELITE CORPORATION, OF NEW YORK, N. Y., A CORPORATION OF DELAWARE

## PREPARATION OF THERMOPLASTIC SHEETS

No Drawing.

Application filed July 5, 1928. Serial No. 290,702.

This invention relates to the production in continuous operation and in sheet form of substantially dry thermoplastic mixtures of a fiber (organic or inorganic) and a synthetic resin of the reactive type. Reactive resins, as is now well understood in this art, are such as are transformed by sufficient application of heat into a hard, strong and infusible state, generally designated as condition C.

10 In the manufacture of thermoplastic sheets according to the present invention, the reactive resin and fiber may first be beaten together in presence of water, and the resulting pulp laid into sheets, in known manner, 15 these operations and the equipment used being somewhat similar to those employed in the manufacture of paper. The excess water is removed on the screens by suction or otherwise as in paper making.

20 In the manufacture of ordinary paper the residual water is readily driven out by passing the yet moist sheet over steam heated rolls, this operation also conditioning the 25 sizing and developing the desired qualities in the paper. But in the production of thermoplastic sheets as herein contemplated, a totally different situation arises, in that the 30 water, or a large portion of it, must be eliminated without materially affecting or injuring the thermoplastic or other characteristics of the resin binder. This result cannot be accomplished by the use of the usual equipment of the paper mill: nevertheless it is essential 35 that the elimination of water should take place rapidly and under conditions affording continuous and large scale production at minimum cost, while leaving the dried sheet in the most serviceable condition for its ultimate applications. Such ultimate applications involve compacting the sheet with or 40 without previous shredding, into such various shapes as plates, slabs, blocks, tubes, gears, and special articles of all kinds, requiring a thermoplastic condition of the 45 binder resin.

A preferred method of accomplishing this result in accordance with the present invention includes subjecting the moist sheet to a stream of dehydrated air or other gas under 50 conditions adapted to effect the rapid re-

moval without injuriously advancing the resin towards condition C or affecting its plasticity. This is best accomplished by first artificially dehydrating the air or other gas either by chemical dehydrating agents such as concentrated sulfuric acid, calcium chlorid or the like; or by physical means, such as refrigerating devices through which the air is directed, preferably in contact with the surfaces of pipes or coils cooled by circulating brine, ammonia or sulfur dioxid or similar refrigerating agents to the point that water vapor content is precipitated as cold water, ice or snow. The dehydrated gas is then heated, as for example by passing it through a bank of steam coils, and is blown upon or over the moving sheet in suitable chambers, tunnels or conduits. It is advantageous to blow the gas against both upper and lower surfaces of the moving sheet, especially if the latter is of considerable thickness. It is likewise advantageous to direct the gas current upon the middle portion of the sheet in such manner that the drying proceeds from the middle outwardly, as any tendency to curling at the edges is thereby minimized.

It has been found that the liability to injury of the sheet is greater while the proportion of moisture present in the sheet is higher; so that somewhat more freedom in the application of heat is permissible as the drying progresses. The temperature of the air or gas may vary considerably according to particular conditions, including the thickness and rate of movement of the sheet, the percentage of moisture therein, the velocity of the gas stream, the special characteristics of the resin binder with respect to plasticity and rapidity of reaction, the particular characteristics desired in the dried sheet, etc. etc. The maximum temperature which may be safely used under any given conditions and for the production of any given product is however readily determined by simple test.

It is important that the actual temperature of the sheet should be kept below the fusing or excessive softening temperature of the resin binder, since fusion or excessive softening is apt to lead to sticking of the sheets and the formation of impervious areas, spots and

55

60

65

70

75

80

85

90

95

100

other defects. It will be understood, however, that the absorption of heat by evaporation of the moisture tends strongly to cool the sheet, so that so long as evaporation is sufficiently rapid, the actual temperature of the dehydrating gaseous medium may be decidedly above the melting point of the resin without injury to the latter. For this reason no definite limitation is placed upon the 10 temperature of the gas, while the temperature of the moving sheet is carefully controlled.

In special cases gaseous media other than air, for example, inert or non-oxidizing gases 15 such as nitrogen, combustion gases, etc. may be used. If desired, the air or gas may be circulated in a closed cycle passing alternately and repeatedly in contact with the moving sheet and the dehydrating means.

20 The extent to which the drying of the sheet is carried in any particular case will of course depend upon the attending circumstances. In general, absolute dehydration of the sheet is not necessary at this stage, since some 25 absorption of moisture may take place in any prolonged period of subsequent storage, unless special precautions are adopted.

The present process is applicable to mixtures containing reactive synthetic resins of 30 all types, although more specially intended for use with reactive resins of the known phenol aldehyde and cresol aldehyde types.

I claim:

1. Process of preparing a substantially dry 35 fibrous sheet containing a synthetic resin in reactive form which comprises the steps of preparing an aqueous suspension of fiber and reactive resin, continuously laying the mixture into a sheet and draining excess water 40 therefrom, dehydrating a current of gas, heating said current of dehydrated gas, and applying said current of heated dehydrated gas to the moving sheet at a rate and a temperature such that the temperature of the sheet 45 remains below that at which excessive softening of the contained resin occurs whereby residual moisture is rapidly removed without substantially injuring the reacting properties of the resin or modifying its plasticity.

50 2. Process of preparing a substantially dry fibrous sheet containing a synthetic resin in reactive form which comprises the steps of preparing an aqueous suspension of fiber and reactive resin, continuously laying the mixture into a sheet and draining excess water 55 therefrom, dehydrating a current of gas, heating said current of dehydrated gas, and passing said current of heated dehydrated gas over at least one surface of the moving sheet at a rate and a temperature such that the temperature of the sheet remains below that at which excessive softening of the contained resin occurs whereby residual moisture 60 is rapidly removed without substantial- 65

ly injuring the reacting properties of the resin or modifying its plasticity.

3. Process of preparing a substantially dry fibrous sheet containing a synthetic resin in reactive form which comprises the steps of preparing an aqueous suspension of fiber and reactive resin, continuously laying the mixture into a sheet and draining excess water therefrom, dehydrating a current of gas, heating said current of dehydrated gas, and passing said current of heated dehydrated gas over both surfaces of the moving sheet at a rate and a temperature such that the temperature of the sheet remains below that at which excessive softening of the contained resin occurs whereby residual moisture is rapidly removed without substantially injuring the reacting properties of the resin or modifying its plasticity. 70 75

4. Process of preparing a substantially dry fibrous sheet containing a synthetic resin in reactive form which comprises preparing an aqueous suspension of fiber and reactive resin, continuously laying the mixture into a sheet and draining excess water therefrom, dehydrating a current of gas, heating said current of dehydrated gas, and passing said current of heated dehydrated gas over at least one surface of the moving sheet, the gas current being directed upon the middle portion thereof at a rate and a temperature such that the temperature of the sheet remains below that at which excessive softening of the contained resin occurs whereby residual moisture is rapidly removed without substantially injuring the reacting properties of the resin or modifying its plasticity, and whereby the drying of the sheet proceeds 80 85 90 95 from the middle outwardly.

5. Process of preparing a substantially dry fibrous sheet containing a synthetic resin in reactive form which comprises the steps of preparing an aqueous suspension of fiber and reactive resin, continuously laying the mixture into a sheet and draining excess water 100 therefrom, heating a current of gas, and passing said current of heated gas over at least one surface of the moving sheet at a rate and a temperature such that the temperature of the sheet remains below that at which excessive softening of the contained resin occurs whereby residual moisture is rapidly removed without substantially injuring the reacting properties of the resin or modifying its plasticity. 105 110 115 120

In testimony whereof, I affix my signature.  
LEO H. BAEKELAND.